

## UNITED STATES PATENT OFFICE

2,210,593

## BEARING ALLOY

William E. McCullough, Detroit, Mich., assignor  
to Bohn Aluminum & Brass Corporation, De-  
troit, Mich., a corporation of Michigan

No Drawing. Application July 31, 1939,  
Serial No. 287,681

2 Claims. (Cl. 75—175)

The invention relates to alloys and more particularly to alloys adapted for use as bearings, as for example a lining in a shell of a different metal.

5 One of the principal objects of the invention is to obtain an alloy which has better properties and characteristics than Babbitt metal. More particularly, it is an object of the invention to obtain an alloy having higher compression strength at elevated temperature, greater resistance to cracking due to fatigue, more effective bonding to the backing metal while at the same time having at least as good resistance to shaft wear as Babbitt.

10 15 My improved bearing alloys are essentially ternary alloys of tin, silver and antimony, although small amounts of other metals may sometimes be present either as impurities or intentionally added.

20 In its broader aspects, my invention comprises alloys having the following analysis:

|    | Per cent    |
|----|-------------|
| Ag | 0.5 to 7.6  |
| Sb | 5.0 to 15.0 |
| Sn | Balance     |

30 However, other metals such as copper, nickel, iron, zinc, cadmium and lead may be present singly or in combination providing the total of these metals is not substantially in excess of 1.5%.

35 As illustrative of my invention, the following specific examples are given:

| 40        | Alloy   | Silver  | Antimony | Tin |
|-----------|---------|---------|----------|-----|
| Example 1 | Percent | Percent | Balance. |     |
| Example 2 | 2.12    | 7.57    |          |     |
| Example 3 | 3.40    | 7.32    | Do.      |     |
| Example 4 | 4.56    | 4.49    | Do.      |     |
| Example 5 | 5.98    | 6.72    | Do.      |     |
|           | 7.51    | 6.89    | Do.      |     |

45 I have observed that the Brinell hardness of my alloys increases with increasing amounts of silver and of antimony. The alloys of the above examples may be prepared without difficulty since the silver and antimony are soluble in molten tin. The alloys may also be made up into composite metal bearings in which the alloys form a liner for bearing shells as of steel, cast bronze or wrought bronze. In preparing such composite bearings, it is desirable to use a flux such as acidified zinc chloride on the shells and then to tin the shells. The tinning may be carried out with pure commercial tin or with an alloy of such tin with up to 15% of lead. Generally speaking, I prefer to use commercially pure tin for the first coating prior to lining with my new alloys.

50 55 60 As before stated, one of the advantages of my new silver alloys is that they have higher com-

pression strength at elevated temperatures than Babbitt alloys containing corresponding amounts of copper. This is illustrated by the following tests which compare the compression strength both at room and elevated temperatures. In carrying out the tests, cylinders of four compositions, A, B, C and D as listed below, were cast in graphite molds and machined to one-half inch diameter and one and one-half inches length.

| 10 | Alloy   | Copper  | Silver  | Antimony | Tin     | Lead | Percent |
|----|---------|---------|---------|----------|---------|------|---------|
| A  | Percent | Percent | Percent | 7.22     | Balance | 0.15 |         |
| B  | 2.12    | None    | 6.79    | do       | do      | 15   |         |
| C  | 3.40    | None    | 7.57    | do       | do      | 10   |         |
| D  | 4.56    | 2.12    | 7.32    | do       | do      | 15   |         |

20 It will be observed in the above table that Babbitt alloys A and B were substantially the same as my new silver alloys C and D except that they had copper instead of the silver of my alloys. The cylinders were tested under compression and the loads determined at 1% permanent reduction in height of the specimens at 70° F. and 300° F.

| 25 | Alloy            | 1% permanent set at 70° F. | 1% permanent set at 300° F. |
|----|------------------|----------------------------|-----------------------------|
| A  | Lbs. per sq. in. | Lbs. per sq. in.           |                             |
| B  | 9550             | 3450                       |                             |
| C  | 9570             | 3350                       |                             |
| D  | 9975             | 4250                       |                             |
|    | 9500             | 4400                       |                             |

30 35 40 From the above, it will be readily apparent that my new silver alloys are at least equal in compression strength at room temperatures to the Babbitt alloys A and B, but are far superior in compression strength at elevated temperatures.

To illustrate another advantage of my alloys, a steel-backed bearing was lined with composition D and fully machined by turning, boring and broaching in a well known manner. The lining metal machined very well and after broaching of the lining had a mirror-like surface, free from porosity, gas holes, oxides or any other defects.

45 50 55 To illustrate another advantage of my alloys the bearing lined with composition D was cut into half shells, flattened with a hammer, and after repeated bendings, it was impossible to separate the silver-antimony-tin lining from the steel shell by use of a chisel or any other means except melting of the lining. By comparison it was possible to separate the lining from a similar bearing lined with composition B with a chisel, the separation occurring between the lining B and the tin coating on the steel backing member.

60 To further illustrate the advantage of my alloys, steel-backed bearings were made according

to conventional production practice to fit a well-known automotive connecting rod. The bearings were tested in a standard and generally used testing machine under conditions of loading, shaft speed, oil temperature and duration to simulate extreme hard conditions of engine operation. Similar bearings lined with composition D were tested under the same conditions.

| 10 | Steel-backed bearing lined with alloy | Shaft speed, R. P. M. | Bearing load, P. S. I. | Time of operation, hours | Oil pressure, P. S. I. | Oil temp., °F. | Bearing temp., °F. |
|----|---------------------------------------|-----------------------|------------------------|--------------------------|------------------------|----------------|--------------------|
| 15 | B-----                                | 1800                  | 437                    | 1                        | 75                     | 207            | 188                |
|    |                                       | 2800                  | 1058                   | 1                        | 75                     | 206            | 185                |
|    |                                       | 3200                  | 1382                   | 1                        | 75                     | 221            | 219                |
| 20 | D-----                                | 3750                  | 1897                   | 1                        | 75                     | 238            | 224                |
|    |                                       | 4000                  | 2159                   | 20                       | 75                     | 273            | 250                |
| 25 | D-----                                | 1800                  | 437                    | 1                        | 75                     | 207            | 240                |
|    |                                       | 2800                  | 1058                   | 1                        | 75                     | 205            | 236                |
|    |                                       | 3200                  | 1382                   | 1                        | 75                     | 210            | 290                |
|    | D-----                                | 3750                  | 1897                   | 1                        | 75                     | 233            | 310                |
|    |                                       | 4000                  | 2159                   | 20                       | 75                     | 242            | 208                |

30 The schedule of oil and bearing temperatures

show the variations normally experienced in such testing, the early variations occurring during the conformation of the bearing surfaces to the shafts. At the end of the tests the bearings were removed. Those lined with alloy B had failed 5 badly due to fatigue cracking of the lining and loosening of pieces of the lining material from the steel back. By comparison, the bearings lined with composition D were still in excellent condition showing practically no fatigue cracks and no 10 loosening of the lining material.

Since the type of bearing failures induced in these tests are known to reliably duplicate in a few hours what would normally occur to bearings after approximately 30,000-40,000 miles of 15 engine operation in an automobile, the superiority of my alloys when used as bearing linings for engines is clearly indicated.

The above tests show that my new silver alloys have physical properties of such a character as to make them more desirable for use as linings in bearing shells than the Babbitt metal of the prior art. Thus by means of my invention I have produced an improved composite bearing.

What I claim as my invention is:

1. A bearing alloy comprising antimony 5 to 15%, silver 0.5 to 7.6% and the balance of tin.
2. A bearing alloy comprising antimony 6.5% to 8.0%, silver 2 to 7.5% and the balance of tin.

WILLIAM E. McCULLOUGH.